

## UNITED STATES PATENT OFFICE

GUY DUNSTAN BENGOUGH AND JOHN McARTHUR STUART, OF LONDON, ENGLAND

## PROCESS OF PROTECTING SURFACES OF ALUMINUM OR ALUMINUM ALLOYS

No Drawing. Application filed July 28, 1924, Serial No. 728,765, and in Great Britain August 2, 1923.

This invention relates to an improved process of producing a resistant coating, by oxidation of the metal when made an anode, on the surface of aluminum or aluminum alloys by anodic treatment in an electrolytic bath.

According to the invention, such a coating is produced by anodic treatment in a bath consisting of an aqueous solution of chromic acid.

10 The conditions of concentration and temperature may be varied accordingly as aluminum itself or any particular alloy of aluminum is under treatment.

In the case of the metal known under the registered trade mark "duralumin" or of commercial sheet aluminum the following directions give the best result at present known to us.

15 The object is first washed in a solvent for grease and then in hot water; it is then made the anode in a bath consisting of an aqueous solution of chromic acid of 3 per cent strength (the chromic acid being calculated as  $\text{CrO}_3$ ), which should be free from sulphuric acid and 20 sulphates. The cathode may be of carbon.

The immersed surface should consist entirely of aluminum or aluminum alloy, the electrical connections being made so that no other metal dips into the bath. If necessary 25 the object may be partially immersed and treated and then inverted so that the remainder of the surface is now immersed and becomes treated.

The temperature of the bath is kept at 40° C. at least and the bulk may be stirred during the treatment. The voltage must be carefully regulated to suit the other conditions; when the latter are those already 35 named the following procedure has been found suitable:—Raise the voltage across the bath gradually to 40 volts in 15 minutes, keep at 40 volts for 35 minutes, and then raise the voltage to 50 volts in the course of 5 minutes 40 and retain it at this value for 5 minutes. The object is then washed and dried.

The film or coating produced by this invention is highly uniform and thicker than those produced by other processes; hence the 45 coated articles when completely immersed in

such liquids as sea-water resist pitting and other forms of attack for long periods.

The degree of resistance is greatly increased if the coated surface is greased or oiled; for the coating has great power of absorption and the grease becomes incorporated in the surface. For this reason the coated surface is well adapted for being painted since the oil of the paint becomes adsorbed. Lanoline is a particularly suitable 55 grease for treating the coated surface; it may be applied in liquid form, in solution or as an emulsion.

As will be clear from the foregoing description, the invention is applicable both to surfaces purely of aluminum and to surfaces comprising aluminum in the form of an aluminum alloy, and it is accordingly to be understood that in the appended claims, the expression "predominantly of aluminum" is intended to include both aluminum itself and 60 alloys of aluminum.

Having thus described the nature of the said invention and the best means we know of carrying the same into practical effect, we claim:—

A process of producing a resistant coating by oxidation on a surface predominantly of aluminum, which process consists in washing the surface with a solvent for grease and then in hot water, making the washed surface the anode in an electrolytic bath consisting of an aqueous solution of chromic acid of 3 per cent strength and containing a carbon cathode, maintaining the temperature of the bath at a temperature not less than 40° C., raising the voltage across the bath to about 40 volts in the course of about 15 minutes, keeping the voltage at this value for about 35 minutes, then raising the voltage to about 50 volts in the course of about 5 minutes and keeping it at this value for about 5 minutes and then washing and drying the surface.

In testimony whereof we have signed our names to this specification.

GUY DUNSTAN BENGOUGH.  
JOHN McARTHUR STUART.